

## UNITED STATES PATENT OFFICE.

JOSEPH W. WEITZENKORN, OF PITTSBURGH, PENNSYLVANIA, ASSIGNOR TO MOLYBDENUM CORPORATION OF AMERICA, OF PITTSBURGH, PENNSYLVANIA, A CORPORATION OF DELAWARE.

## STEEL ALLOY.

No Drawing.

Application filed March 30, 1926. Serial No. 98,618.

In United States Patent No. 1,401,926, granted to George W. Sargent and me, there is disclosed a manganese steel alloy to which molybdenum is added with the result that 5 the usual physical properties of manganese steel are intensified and its range of heat treating temperatures greatly increased without developing brittleness. The resulting manganese steel so disclosed contains not 10 more than about .80 per cent carbon, from about 1.15 to 3.00 per cent manganese, and from about 1.00 to 1.25 per cent molybdenum, the remainder being iron with the exception of impurities and other elements 15 customarily found in steel as the result of manufacturing processes.

The present invention relates to alloys such as disclosed in said patent, and is predicated upon my discovery that by increasing 20 the carbon content of the alloy there is produced an alloy having the characteristics of both iron and steel, and which is particularly suitable for the manufacture of hot work articles, such as rolls for steel mills, 25 dies for forgings, etc.

The alloy provided according to this invention contains from about .85 to 2.50 per cent carbon, from about 1.15 to 3.00 per cent manganese, and from a fraction of one per 30 cent to 1.25 per cent molybdenum, the remainder being iron except for the usual amounts of other elements, such as sulphur, phosphorus, silicon and the like, which are ordinarily present as impurities or as in-

cidental to manufacturing processes. The sulphur and phosphorus should be as low as possible, while silicon and the like may be present to the extent usually found in most steels.

The alloy resembles iron in that it is very 40 hard and wear-resisting, and it resembles steel in that it is tough, strong and dense. In addition to these characteristics, the alloy is highly resistant to fire cracking, which, coupled with its hardness, renders it 45 particularly well suited for use in the manufacture of hot work articles, such as have been mentioned.

In the manufacture of this alloy, it has been found advantageous to heat the molten 50 metal to a high temperature, for example from about 2800 to 3000° F., while in a furnace, and to cast it from as low a temperature as is commercially possible. In its solid state it may be heat treated throughout 55 a wide range of temperatures without developing brittleness.

I claim as my invention:

A steel alloy containing from about .85 to 2.50 per cent carbon, from about 1.15 to 60 3.00 per cent manganese and from a substantial fraction of one per cent to 1.25 per cent molybdenum, the remainder being iron except for the usual amounts of other elements present as impurities or as incidental to 65 manufacturing processes.

In testimony whereof, I sign my name.  
JOSEPH W. WEITZENKORN.